



zontal. The wire was seated in a bottomless wooden box so arranged that the fine fibres passing through the wire were collected in a fine muslin cloth directly below the wire, while the coarser fibres could be washed down the incline into another fine muslin cloth. The pulp retained on the wire was picked up and diluted in a pail and again poured over the wire. This operation was repeated until no more fines passed through. The fines were not considered acceptable for bleaching, but were dried and weighed separately. The weight of the fines was included in the total yield of unbleached pulp. After the foregoing procedure was carried out, the remaining pulp was left standing over night before the final washing step, but this is optional. For final washing the accepted pulp was placed in a beater and circulated for thirty minutes, using a balanced bedplate.

At the conclusion of the beating period, the pulp was removed from the beater and washed down the inclined screen to remove any additional fines which the beating might have dislodged. The pulp retained on the wire after the second washing operation was considered satisfactory for bleaching.

A portion of this "accepted pulp" was then bleached using hypochlorite solution containing (based on the accepted pulp) 7.5% of available chlorine.

Test figures for the foregoing operations are as follows:

| Evaluation Data                           | Per cent |
|-------------------------------------------|----------|
| Total unbleached yield                    | 47.9     |
| Accepted pulp yield (fines removed)       | 22.3     |
| Bleaching loss (based on acceptable pulp) | 4.6      |
| Alpha-cellulose in unbleached pulp        | 89.6     |
| Alpha-cellulose in bleached pulp          | 86.8     |

It will be noted that there was degradation of the pulp from 89.6 to 86.8% during the bleaching step which was carried out in the absence of the inhibiting ingredients—viz. ammonium hydroxide potassium carbonate and ammonium oxalate—in the bleaching solution.

#### Example 2

1 ton of air-dry cotton seed hulls (after soaking in water for 14 hours) were digested for about 2 hours in a solution made up as follows:

|                                        |  |
|----------------------------------------|--|
| 20,000 lbs. water                      |  |
| 480 lbs. NaOH                          |  |
| 20 lbs. NH <sub>4</sub> OH of 26° Bé.  |  |
| 30 lbs. K <sub>2</sub> CO <sub>3</sub> |  |
| 10 lbs. ammonium oxalate (cryst.)      |  |

The digestion was at 300° to 350° F. (= 149° to 177° C.) under pressure. During this treatment most of the hull proper (horny seed coat) was dissolved.

The pulp was washed, screened as above to remove fines, and dried. Yield of cellulose pulp was good. It will be noted that here, the ratio of water to cotton seed hull was 10:1, and the NaOH was equal to 24% of the weight of the cotton seed hulls. The NaOH in the solution was about 2.34%, and the total chemicals in the solution was about 2.63%.

A similar test, with the above materials in the same proportions in which the digestion time was 2½ hours gave similar results, and a fairly good yield.

A considerable portion of the caustic soda was used up in attacking the hard seed coat. It is on

this account that the percentage of NaOH (based on the hulls) is large.

#### Example 3

Three ounces (85 grams) of air-dry cotton seed hulls (2 years old) were placed in a steam jacketed autoclave with a digesting solution which comprised 64 ounces (½ gal. or about 1.9 liters) of water in which had been dissolved 17 grams of caustic soda, 0.08 gram of 26° Bé. ammonia water, 0.12 gram of potassium carbonate and 0.04 gram of ammonium oxalate. The autoclave was sealed and steam under pressure admitted to the jacket. During cooking, the steam pressure varied from 100 to 135 lbs. However, the temperature within the digester was maintained at a mean temperature of 335 degrees F. (i. e. about 170° C.) for a period of three hours. At the conclusion of this cooking period the autoclave was vented to gradually reduce the pressure within the same. It was noticed that there was an absence of ammonia in the steam and other gases which escaped from the autoclave when it was vented. The pulp was removed from the autoclave and carefully washed and then dried. When thoroughly dried it was carefully weighed and a yield determination made. It was found that the yield was slightly over 50% (based on the cotton seed hulls treated).

While I have given above the ingredients and relative proportions of ingredients to obtain good yields of alpha cellulose pulp with desirable characteristics from cotton seed hulls, it will be apparent to those skilled in the art that the proportions and amounts of chemicals to be used may in some instances be varied, depending upon the kind, quality, condition and state or source of supply of the raw cotton seed hulls available. In practice and based upon many tests and experiments which I have made, the proportions and ingredients for digesting and cooking cotton seed hull may vary as follows and yet afford the most advantageous results in the described process.

When cotton hulls are digested, the proportions and amounts of the ingredients per ton of hulls may be varied as follows, while affording very advantageous results in the described process, both as to yield and quality of cellulose.

|                                                                                    |           | Pounds per ton |
|------------------------------------------------------------------------------------|-----------|----------------|
| NaOH (alone or with carbonate),                                                    |           |                |
| 16½ to 24%                                                                         | 330 to    | 480            |
| Water, about 500% to 1200%                                                         | 10,000 to | 24,000         |
| NH <sub>4</sub> OH (26° Bé.), 1½ of 1% to 1%                                       | 13¾ to    | 20             |
| K <sub>2</sub> CO <sub>3</sub> (98%), 1¾ to 1½—                                    | 20% to    | 30             |
| (NH <sub>4</sub> ) <sub>2</sub> C <sub>2</sub> O <sub>4</sub> (crys. c. p.), 1½ to |           |                |
| ½%                                                                                 | 6% to     | 10             |

By the foregoing process, cotton seed hulls can be processed so as to obtain relatively high yields of cellulose pulp. The pulp also has a high alpha cellulose content. By carrying out the digesting operation in the presence of ammonium hydroxide, potassium carbonate and ammonium oxalate, degrading of the cellulose which tends to take place under the action of the relatively strong alkaline digesting solution is restrained. It is not intended to imply by the inclusion in the summary table above, that the ammonium hydroxide must be added as "26° Bé." ammonia water (i. e., containing 28% NH<sub>3</sub> in solution), but that the amount of ammonia solution used is equivalent to the stated amount of 26° ammonia. Similarly the reference to "98% calcined" in referring to the potassium carbonate, and the ref-

erence to "crys. c. p." in referring to the ammonium oxalate, are for showing that the amounts (pounds) of these substances are calculated on these bases. The alpha cellulose obtained also has the desirable characteristics which are shown by test data figures.

In the above examples, I have stated preferred temperatures, pressures and times of treatment, which have been found to be satisfactory. It is not desired, however, to limit the invention to these details, since it will be apparent to those familiar with the art, that these features are subject to variation. In most cases, I prefer to maintain the temperature during the cooking, at about 160° to 170° C., although the temperature may fluctuate over a somewhat wider range. After the heating up, the liquor is at or near its boiling point (under the existing pressure). In many runs, temperatures between 156° and 172° C. have given good results. The time during which these temperatures are maintained is also variable; times 2, 2½ and 3 hours are given in the examples, as suitable. But it will be understood that the cooking is to be continued until the cellulose fibre is sufficiently loosened, and until the hard seed coat is dissolved or disintegrated. This is generally a few hours. The pressures obviously will be dependent on the temperature of the cooking operation, since the pressure is developed by the boiling of the solution or liquor in the digester and the liberation of vapors therefrom. In the examples, I have mentioned, by way of example, pressures of 52 lbs. to 135 lbs., per square inch, as being suitable. Generally, with a given material (seed hulls and solution) to be digested, high pressure will be produced by high temperature, and vice versa.

Cotton seed hull, in air-dry condition may contain about 7 to 10% of moisture. These figures will vary somewhat depending on the atmospheric conditions during the drying and storage of the materials in question.

Operating in accordance with Example 1 above, I have made alpha cellulose of 95% purity, having very satisfactory properties for use in making such products as nitrocellulose (for explosives).

The "cotton seed hulls" carries a substantial amount of short fibered cotton fuzz attached to pieces of the hard, horny seed coat, the latter component amounting to roughly one half (50%) of the said material, and horny seed coat as is well known, does not contain but a very small percentage of alpha cellulose. This "seed coat" or actual hull of the seed has to be substantially all dissolved in the cooking liquor, during the digestion. Thus it will be seen that the material treated in the present process is radically different from "cotton seed hull fibre" treated as starting material in the copending case 605,639.

I claim:

1. A process of making cellulose of high alpha content from cotton seed hulls carrying a fuzz of cotton seed hull fibres rigidly attached to broken pieces of the seed coat itself, which process comprises first soaking said material in water for at least several hours, then digesting such hulls in a closed pressure tight digester, under about 52 lbs. to about 135 lbs. pressure and at approximately 149° to 177° C., in an aqueous solution containing from 2.34% to 3.46% of caustic soda as its main chemically active dissolved constituent, together with an inhibitor of degrading of the cellulose, which inhibitor consists essentially of one part of ammonium oxalate, about two parts of

ammonium hydroxide calculated as 26° Bé. and about three parts of potassium carbonate, the amount of said inhibitor being from about one-tenth to about one-sixth of the amount of said caustic soda, the amount of caustic soda being approximately 16.5 to 24%, based on the air-dry weight of the said cotton seed hulls, and continuing said digestion until the said pieces of seed coat are substantially all separated from the cotton seed hull fibres and disintegrated.

2. A process of obtaining alpha cellulose from cotton seed hulls carrying cotton seed hull fibre rigidly attached thereto, which comprises digesting the premoistened hulls under pressure and at a temperature of about 171° C. in a digesting solution containing the following ingredients expressed in pounds per ton of air-dry hulls:

360 pounds of sodium hydroxide  
15 pounds of ammonium hydroxide (26° Bé.)  
22.5 pounds potassium carbonate  
7.5 pounds ammonium oxalate  
10,000 pounds water

and continuing such digestion for a period of about 3 hours and until the seed coat component is substantially all dissolved.

3. A process of obtaining alpha cellulose from cotton seed hulls carrying cotton seed hull fibre rigidly attached thereto, which comprises digesting the premoistened hulls under super-atmospheric pressure, and at a temperature of about 149° to 177° C. in a digesting solution containing the following ingredients expressed in pounds per ton of air-dry hulls:

35 480 pounds of sodium hydroxide  
20 pounds of ammonium hydroxide (26° Bé.)  
30 pounds potassium carbonate  
10 pounds ammonium oxalate  
40 20,000 pounds water

and continuing such digestion for a period of about 2 hours and until the seed coat component is substantially all dissolved.

4. A process of obtaining alpha cellulose from cotton seed hulls carrying cotton seed hull fibre rigidly attached thereto, which comprises digesting the premoistened hulls under pressure and at a temperature of about 156° to 172° C. in a digesting solution containing the following ingredients expressed in pounds per ton of air-dry hulls:

45 360 to 480 pounds of sodium hydroxide  
About 15 to about 20 pounds of ammonium hydroxide (26° Bé.)  
55 About 22.5 to about 30 pounds of potassium carbonate  
About 7.5 to about 10 pounds ammonium oxalate  
About 10,000 to about 20,000 pounds water

60 in which digesting solution the sodium hydroxide content amounts to between 2.34% and 3.46% and the sodium hydroxide is between 6 and 10 times the combined amounts of ammonium oxalate, 26° Bé. ammonia water and potassium carbonate, and continuing such digestion for a period of about 2 hours and until the seed coat component is substantially all dissolved.

5. In the art of digesting cotton seed hulls carrying a fuzz of cotton fibres rigidly attached to broken pieces of the seed coat itself, in caustic soda lye, of about 2.34% to about 3.46% concentration, under a superatmospheric pressure of about 52 pounds to about 135 pounds per square inch, and at approximately the boiling point of the said lye under the existing pressure, until said

pieces of seed coat become substantially all disintegrated, the herein described improvement which consists in adding to said lye an inhibitor to inhibit the degradation of alpha cellulose present in said fuzz, which inhibitor contains about 1 part ammonium oxalate, about 2 parts of ammonia calculated as 26° Bé, ammonia solution and about 3 parts of potassium carbonate, one part of said inhibitor being added to each 6 to 10 parts of caustic soda in said lye.

6. As a new composition of matter, a digestive solution which is a solution containing as its essential constituents, dissolved in water,

|                                                    | Parts |
|----------------------------------------------------|-------|
| Ammonium oxalate                                   | 1     |
| Ammonium hydroxide, calculated as 26° Bé,<br>about | 2     |
| Potassium carbonate, about                         | 3     |
| Caustic soda, about                                | 48    |

the percentage of caustic soda in such solution being between about 2.34 and about 3.46.

JEFFERSON L. ESKRIDGE.

#### REFERENCES CITED

The following references are of record in the file of this patent:

#### UNITED STATES PATENTS

|    | Number    | Name    | Date          |
|----|-----------|---------|---------------|
| 10 | 1,842,649 | Bassett | Jan. 26, 1932 |
|    | 1,998,344 | Thomas  | Apr. 16, 1935 |

#### FOREIGN PATENTS

|    | Number  | Country       | Date          |
|----|---------|---------------|---------------|
| 15 | 347,444 | Great Britain | Apr. 30, 1931 |